

Feb. 14, 1961

T. A. DUNTON ET AL  
IRON POWDER AND THE MANUFACTURE OF  
MAGNETIC CORES THEREFROM  
Filed Nov. 27, 1957

2,971,872



Fig.1.



Fig.2.



Fig.3.

THORNLEY ATELSTANDUNTON  
DAVID KENNETH WORN  
*Inventors*

By *C. Jr. Diller*  
Attorney

# United States Patent Office

2,971,872

Patented Feb. 14, 1961

1

2,971,872

## IRON POWDER AND THE MANUFACTURE OF MAGNETIC CORES THEREFROM

Thornley Athelstan Dunton and David Kenneth Worn, Birmingham, England, assignors to The International Nickel Company, Inc., New York, N.Y., a corporation of Delaware

Filed Nov. 27, 1957, Ser. No. 699,285

Claims priority, application Great Britain Sept. 16, 1954

2 Claims. (Cl. 148—105)

The present invention relates to magnetic cores used at very high frequencies as well as to a special iron powder used in making these magnetic cores, and more particularly to a carbonyl iron powder, the fine particles of which have aggregated during decomposition of the carbonyl to form an open mesh and hereinafter termed "fibrous" powders, of improved electromagnetic properties for use in high frequency electromagnetic cores.

It is well known that the manufacture of metal powders from their carbonyls was originally developed by Mond in 1890. The use of this powder for electrical purposes by the Germans during World War II has been described in British Intelligence Objectives Sub-Committee (B.I.O.S.), Final Report No. 1575 (Interrogation of Dr. Leo Schlecht, pages 20-28). Carbonyl iron powder is presently used to make magnetic cores for induction coils for use at very high frequencies. It is often important for very high frequency use that the coils be high "Q" coils and that the core of the coil increases the "Q" or merit of the coil. The "Q" of a core coil assembly is defined as the ratio of the inductive reactance to the effective resistance and can be expressed as follows:

$$Q = wL/R_e$$

where  $L$  is the inductance in henries,  $w$  is  $2\pi \times$  frequency in cycles per second and  $R_e$  is the total effective resistance.

$R_e$  comprises not only the resistance of the winding,  $R_w$ , but also the effective resistance caused by eddy-current, hysteresis and other losses occurring in the core when the latter is in an alternating field. The winding resistance at the test frequency may be written as

$$R_w = R_{D.C.}(1+\alpha)$$

where  $\alpha$  is a function of frequency, coil shape, wire size and resistivity. The contribution of  $R_{D.C.}$  to the total losses is reduced in proportion to the effective permeability and physical size of the core, but the core losses increase with permeability, thus a suitable compromise has to be made.

It has been established that in weak fields (such as usually obtain in communication engineering, e.g. up to about 10 oersteds) the A.C. losses introduced by the core can be expressed in the form:

A.C. effective resistance in ohms,

$$R = fLu_c(aB_m + c + ef)$$

where

$f$  is the frequency in cycles per second

$L$  is the effective inductance in henries

$U_c$  is the core permeability

$B_m$  is the maximum flux density in gauss

$a$  is the hysteresis loss constant

$c$  is the residual loss constant

$e$  is the eddy current loss constant

To this must be added the A.C. resistance of the coil. It will be noted that for low frequency applications the principal core losses are the residual and hysteresis losses. At very high frequencies, eddy current losses are pre-

2

ponderant and it is these which usually limit the quality of cores at these frequencies.

In many radio-communication applications, the field strength is very low and from the above expression it is easily seen that the contribution of hysteresis to the total losses is very small indeed.

In our copending application Ser. No. 534,398, filed September 14, 1955, now abandoned, we have explained that magnetic cores used at very high frequencies are commonly made of iron powder produced by the thermal decomposition of iron carbonyl, this powder being commonly called carbonyl iron powder. We have also explained that the size of the powder particles is important, and as the frequency at which the core is used increases it becomes more and more desirable to use as fine a powder as possible.

In the usual method of manufacture, the powder, before being compressed into cores, is mixed with insulating material, which forms insulating layers between the powder particles, and generally also with an additional binder to increase the mechanical strength of the core. The insulating material may be, for instance, sodium silicate, and the binder a phenol-formaldehyde resin. It is well known that the magnetic properties of the cores are greatly influenced by the degree and character of insulation between the particles. When the powders are very fine, having a large proportion of particles of a size well below 3 microns (as determined by a Fisher sub-sieve sizer) difficulties are encountered in insulating them. In particular, if the same percentage of insulation is used as with larger particle powders, the film of insulation, being thinner, tends to break down during pressing, causing particle-to-particle contact.

According to the above-mentioned B.I.O.S. Final Report No. 1575, page 21, the grade E and the grade EN powders described therein are the powders used for high frequency application. The letter "N" after the "E" signifies that the powder had been ball milled. Grade E powder particles are mostly spherical in shape. A photograph of this grade E powder appears in Goetzel, "Treatise on Powder Metallurgy," volume II, 1950, ed., Interscience Pub. Inc., N.Y., page 293. It is exceedingly difficult to produce grade E spherical powder below 3 microns. The usual procedure used for obtaining small particle size powder consists in separating a fine fraction from a spherical powder having a higher average particle size. When attempting to make powders below 3 microns directly in the decomposer, it is often found that although the particle size as determined by a Fisher sub-sieve sizer is indeed below this value, the individual particles are often aggregates of particles of even finer particle size, the overall dimensions of the open mesh being greater than 3 microns. Because of this fibrous nature, it is extremely difficult to properly insulate these particles and part of the invention in our previous patent application Ser. No. 534,398, filed September 14, 1955, as shown particularly in Example I thereof, consists essentially in forming an iron sulfide film on the surface of the fibrous particles, this film improving the electrical insulation between the irregular shaped particles. This treatment improved the "Q" values of cores considerably, but naturally the further elimination of unwanted eddy currents which are a great disadvantage is desirable.

It has now been discovered that a powder consisting of fibrous aggregates of primary particles may be so milled or further milled after the formation of the iron sulfide film as to break up at least a substantial proportion of the clusters or aggregates without breaking up the primary particles themselves to any substantial extent. We find that the Q values of the resultant cores made from

## 3

these fibrous powders are improved, particularly at high frequencies.

It is an object of the present invention to provide a fibrous carbonyl iron powder with exceedingly high Q values when formed into a core for use with an induction coil.

Other objects and advantages will become apparent from the following description taken in conjunction with the drawings in which:

Figure 1 is a reproduction of a photomicrograph taken at 3500 magnification showing the structure of unmilled fibrous powder particles.

Figure 2 is likewise a reproduction of a photomicrograph taken at 3500 magnification showing the structure of unmilled fibrous powder particles.

Figure 3 is a reproduction of a photomicrograph taken at 3500 magnification showing the structure of milled fibrous powder particles produced in accordance with the invention.

Generally speaking, the present invention contemplates the production of iron cores for induction coils useful in very high frequency application by producing fibrous powder in a carbonyl decomposer, insulating the powder with hydrogen sulfide, ball milling the powder, mixing the powder with sodium silicate and a binder and making a core.

5

charge of steel balls weighing over 5 times as much as the powder charge.

The Q values obtained from cores made of the unmilled and milled powder respectively were as follows:

|                 | Pressure,<br>tons/sq. in. | Q values at frequencies (in<br>mc./s.) of— |    |     |     |     |
|-----------------|---------------------------|--------------------------------------------|----|-----|-----|-----|
|                 |                           | 20                                         | 30 | 50  | 100 | 200 |
| Unmilled powder | 20                        | 8                                          | 7  |     |     |     |
|                 | 45                        | 8                                          | 7  |     |     |     |
| Milled powder   | 20                        | 178                                        |    | 161 | 75  | 52  |
|                 | 45                        | 52                                         |    | 27  | 11  | 12  |

10

Other batches of the powder were sulfided in conical flasks by passing hydrogen sulfide gas over them for 2, 3.75 and 4 minutes approximately giving sulfur contents of 0.33%, 0.99% and 1.12%. Part of each batch of sulfided powder was milled in the same way as the starting powder. In addition, part of the batch of milled starting powder was sulfided to a sulfur content of 0.74%, and some of this milled and sulfided powder was then again milled for 16 hours.

20

The Q values obtained from cores made from the powder after these various treatments were as follows:

| Pressure,<br>Tons/sq. in. | Percent<br>Sulfur | After Sulfiding |              |               |               | After sulfiding and Milling |              |               |               |
|---------------------------|-------------------|-----------------|--------------|---------------|---------------|-----------------------------|--------------|---------------|---------------|
|                           |                   | 20<br>Mc./s.    | 50<br>Mc./s. | 100<br>Mc./s. | 200<br>Mc./s. | 20<br>Mc./s.                | 50<br>Mc./s. | 100<br>Mc./s. | 200<br>Mc./s. |
| 20                        | 0.33              | 187             | 218          | 113           | 84            | 192                         | 247          | 140           | 103           |
|                           |                   | 155             | 121          | 52            | 38            | 190                         | 216          | 113           | 80            |
| 20                        | 0.99              | 178             | 224          | 120           | 89            | 185                         | 247          | 150           | 115           |
|                           |                   | 162             | 150          | 72            | 55            | 185                         | 222          | 126           | 98            |
| 20                        | 1.12              | 177             | 185          | 93            | 69            | 188                         | 248          | 154           | 121           |
|                           |                   | 99              | 65           | 29            | 26            | 185                         | 218          | 119           | 92            |
| 20                        | 0.74              | 186             | 243          | 138           | 99            | 189                         | 253          | 150           | 113           |
|                           |                   | 183             | 231          | 123           | 89            | 186                         | 232          | 129           | 98            |

40

From the two tables given above it will be seen that milling alone produced a very marked improvement in the Q values at all frequencies, but that at all the higher frequencies this improvement in itself was not nearly as great as that produced by sulfiding, and milling the powder.

45

The invention is particularly applicable to directly produced fibrous powders having very fine primary particles to be made into cores for use at high frequency.

50

It is to be observed that the present invention provides producing fibrous carbonyl iron powder with a mean particle size of 2.45 microns directly from a carbonyl decomposer, sulfiding the powder, ball milling the powder, mixing the powder with sodium silicate as a further insulating material and a phenol-formaldehyde resin binder and compressing the powder into a core having a high Q and useful at very high frequencies.

55

Furthermore, the invention provides the ball-milling to be done either after the sulfiding treatment or before and after the sulfiding treatment.

60

Moreover, the invention provides sulfiding the powder by passing hydrogen sulfide gas over the powder for from 2 to 4 minutes approximately giving a sulfur content of from 0.33% to 1.12%.

65

The present application is a continuation-in-part of our copending application Serial No. 534,398, filed September 14, 1955.

70

Although the present invention has been described in conjunction with preferred embodiments, it is to be understood that modifications and variations may be resorted to without departing from the spirit and scope of the invention, as those skilled in the art will readily understand. Such modifications and variations are considered to be within the purview and scope of the invention and appended claims.

We claim:

1. In a method for making electromagnetic cores for

In carrying the invention into practice, it has been found that good results may also be obtained by sulfiding the powder, then ball milling the powder, then insulating the powder with sodium silicate, adding an acetone solution of phenol-formaldehyde resin as a binder and compressing the resultant powder mixture into a core, which may take a convenient form such as a cylinder.

For the purpose of giving those skilled in the art a better appreciation of the advantages of the invention, illustrative examples are given below.

The improvements produced are shown by comparative tests in which batches of a single starting fibrous powder were differently treated and formed into cores, the Q values of the cores at various frequencies then being ascertained.

The starting fibrous powder had a mean particle size of 2.45 microns, and was produced directly by decomposition of carbonyl in a decomposer and contained 2.57% carbon, 1.03% nitrogen and 0.001% sulfur. The method employed in making each core consisted of stirring the powder in an insulating material such as an aqueous solution of sodium silicate at about 60° C. until the mixture was dry, adding an acetone solution of a phenol-formaldehyde resin and again stirring until the acetone had evaporated; forming the powder, which contained 1% sodium silicate and 3% resin, into cylindrical cores under pressure; and finally heating at 130° C. for 2 hours to polymerise the resin. Two cores were made from the starting powder and two from each treated powder, one core in each pair being pressed at 20 tons per square inch and the other at 45 tons per square inch.

The starting powder had very poor insulating characteristics and cores made from it had very low Q values even at low frequencies. One batch of the starting powder was milled in a 2 inch diameter and 2 inch long ball mill for 16 hours in a mill containing 1/4 inch diameter steel balls and rotating at 70 revolutions per minute, the

induction coils wherein the cores are pressed from iron powder mixed with a aqueous solution of sodium silicate and a phenol-formaldehyde resin binder, the improvement which comprises sulfiding a fibrous carbonyl iron powder having a mean particle size below about 3 microns with hydrogen sulfide gas to a sulfur content of from 0.3% to 1.2% by weight of iron powder for a period of time of from about 2 minutes to about 4 minutes, and subjecting the powder to a ball milling treatment with a charge of steel balls weighing over 5 times the weight of the powder, whereby higher Q values at very high frequencies are obtained in cores made therefrom.

2. In a method for making electromagnetic cores pressed from iron powder, the improvement which comprises ball milling a fibrous carbonyl iron powder having a mean particle size below about 3 microns with a charge of steel balls weighing over 5 times the weight of the

15 powder, sulfiding the ball milled powder with hydrogen sulfide gas to a sulfur content of from 0.3% to 1.2% by weight of iron powder for a period of time of from about 2 minutes to about 4 minutes and thereafter again subjecting the powder to a ball milling treatment with a charge of steel balls weighing over 5 times the weight of the powder, whereby higher Q values at very high frequencies are obtained in cores made from the thus-treated powder mixed with sodium silicate and a phenol-formaldehyde resin binder.

## References Cited in the file of this patent

## UNITED STATES PATENTS

|           |                |               |
|-----------|----------------|---------------|
| 1,669,648 | Bandur         | May 15, 1928  |
| 2,399,019 | Grinter et al. | Apr. 23, 1946 |
| 2,666,724 | Beller         | Jan. 19, 1954 |
| 2,791,561 | Beller et al.  | May 7, 1957   |